

## UNITED STATES PATENT OFFICE

2,286,867

## MAGNESIUM BASE ALLOY

John C. McDonald, Midland, Mich., assignor to  
The Dow Chemical Company, Midland, Mich.,  
a corporation of Michigan

No Drawing. Application December 23, 1940,  
Serial No. 371,372

2 Claims. (Cl. 75—168)

The invention relates to magnesium base alloys and more particularly concerns an alloy of this nature having an exceptionally high degree of formability associated with other desirable physical properties, such as high tensile and yield strengths.

Magnesium base alloys are being widely used in the structural arts where a light weight metal is highly desirable, such as for use in making castings, forgings, and the like. However, the use of these alloys in the rolled form to make sheet metal articles requiring forming operations, such as bending, drawing, and the like, has not progressed as rapidly due to the fact that, in general, alloys having good formability or ductility permitting relatively sharp bends to be made without the article developing external

that in general the preferred composition range is that in which cerium is present in an amount from about 0.1 to 0.7 per cent, calcium from 0.05 to 0.5 per cent, and cadmium from 3 to 7 per cent. A particularly desirable composition because of its desirable combination of properties is one containing 0.4 per cent of cerium, 0.2 per cent of calcium, and 5 per cent of cadmium.

The following table, listing some of the properties of rolled sheet metal made from my new quaternary alloy and comparing these properties with those of related parent alloys, illustrates the improvement in formability as well as yield and tensile strengths over that of related alloys. In the table the per cent elongation is to be regarded as a measure of the ductility or formability of the alloys.

Table

| Nominal composition in per cent<br>(magnesium=remainder) |      |     | Annealed                       |                               |                                 | Cold rolled                   |                                 |
|----------------------------------------------------------|------|-----|--------------------------------|-------------------------------|---------------------------------|-------------------------------|---------------------------------|
| Ce                                                       | Ca   | Cd  | Percent elongation in 2 inches | Yield strength in lbs./sq.in. | Tensile strength in lbs./sq.in. | Yield strength in lbs./sq.in. | Tensile strength in lbs./sq.in. |
| 0.11                                                     | 0.20 | 5.0 | 15                             | 16,000                        | 31,000                          | 31,000                        | 36,000                          |
| 0.19                                                     | 0.24 | 4.9 | 18                             | 17,000                        | 33,000                          | 32,000                        | 40,000                          |
| 0.11                                                     | 0.08 | 5.0 | 18                             | 20,000                        | 34,000                          | 29,000                        | 36,000                          |
|                                                          |      |     | 21                             | 22,000                        | 36,000                          | 31,000                        | 39,000                          |

cracks, usually have inferior characteristics as regards their tensile and yield strengths.

It is, accordingly, the principal object of the invention to provide a magnesium base alloy which can be made into rolled sheet and the like possessing a sufficient degree of ductility or formability at ordinary temperatures to be sharply bent, drawn or otherwise shaped, while having excellent tensile and yield strengths.

Other objects and advantages will be apparent as the description of the invention proceeds.

My invention resides in the discovery that a magnesium base alloy containing from about 0.01 to 1 per cent of cerium, from 0.01 to 1 per cent of calcium, and from 1 to 12 per cent of cadmium possesses the aforementioned desirable properties. The term "magnesium" used herein and in the appended claims is intended to include magnesium containing the ordinary impurities that are found in the commercially pure metal, such as traces of iron, copper, nickel, and silicon. While the properties of improved ductility or formability associated with high tensile and yield strengths are manifest over the entire range of composition indicated, I have found

the properties set forth above under the term "annealed" were obtained by first rolling the alloys at a temperature of 550° F. and thereafter annealing them at various temperatures through a range of from 400 to 800° F. The properties selected for the table were those of the annealed specimens which exhibited the maximum elongation. The properties set forth under the term "cold rolled" were obtained by subjecting specimens of the alloys which had first been hot rolled at a temperature of 550° F. to additional rolling in the cold state. The properties selected for the table were those of the cold rolled specimens which showed the highest tensile and yield strengths, while having at least a 1 per cent elongation in 2 inches.

A comparison of the properties listed in the table shows that all of the combined properties of my quaternary alloy are always superior to those of related alloys. For example, it will be noted that the new alloy shows superior elongation as well as an improvement in yield and tensile strength. This improvement is present in both the cold rolled and annealed state. Similarly, the improvement illustrated by the partic-

ular composition shown in the table is exhibited throughout the percentage range of alloying ingredients indicated.

While the new alloy is most useful in wrought form, such as sheets, due to its formability characteristics, it may also be used for making castings, extruded forms, and the like.

The new alloy may be compounded by any of the methods usually employed for melting and alloying metals with magnesium such as by adding the alloying ingredient singly or jointly to a bath of molten magnesium which is preferably protected from oxidation by suitable flux. The flux should be substantially free from magnesium chloride, if the calcium content of the alloy is above 0.3 per cent. In those instances where the alloy is to be compounded containing less than 0.3 per cent of calcium, magnesium chloride may be present in the flux, but in this case it is preferable to add the calcium last without too much stirring and agitation in order to prevent loss of calcium into the flux. Cerium

5 may be added to the alloy as such, or in the form of Misch-metal. Magnesium-cerium alloys are commonly made up by employing Misch-metal as a source of cerium. It is sometimes desirable to add more than the theoretical amount of Misch-metal since the alloying efficiency is not always 100 per cent and some loss may be incurred.

10 It is to be understood that the invention is not limited to the particular composition described herein, but may take other forms without departing from the scope of the invention.

I claim:

15 1. A magnesium base alloy containing from 0.1 to 0.7 per cent of cerium, 0.05 to 0.5 per cent of calcium, and from 3.0 to 7.0 per cent of cadmium, the balance being magnesium.

20 2. A magnesium base alloy containing 0.4 per cent of cerium, 0.2 per cent of calcium, 5.0 per cent of cadmium, the balance being magnesium.

JOHN C. McDONALD.